

Nov. 22, 1932.

M. L. MESA

1,888,969

FROSTING PROCESS

Filed March 19, 1950

Fig. 1.



Fig. 2.



Fig. 3.



Fig. 4.



Fig. 5.



Maria Luisa Mesa  
INVENTOR

BY *Victor J. Evans*  
ATTORNEY

WITNESS:

*J. Mank*

## UNITED STATES PATENT OFFICE

MARIA LUISA MESA, OF NEW YORK, N. Y.

## FROSTING PROCESS

Application filed March 19, 1930. Serial No. 437,230.

This invention relates to processes for treating fabrics or other materials or articles in which it is desired to produce a sparkling or frosted effect with the object of making 5 the fabric, material or article more pleasing to the eye, particularly in the case of artificial flowers, tassels, lace, ornaments of various kinds, and the like, such for instance, as shown and referred to in my co-pending application Serial No. 332,092 filed January 12th, 1929.

The primary object of the present invention is to provide a process of the nature specified which involves treating the fabric, material or article with a solution of a salt in which the fabric or the like is dipped and allowed to dry, the salt forming crystals adhering to the fabric or the like after the solvent has evaporated, several such treatments being carried out in order to create varying effects or to secure larger crystals, the composition and nature of the solution being such that the crystals adhere firmly to the fabric or article.

Other objects and advantages of the invention will be hereinafter specifically pointed out, or will become apparent, as the specification proceeds.

With the above indicated objects in view, the invention resides in certain novel steps and order of steps clearly described in the following specification and illustrated in the accompanying drawing, in which:

Fig. 1 illustrates an ornament comprising 35 a butterfly which has been treated by the herein described process.

Fig. 2 is a greatly enlarged section of a piece of fabric which has been treated in accordance with the first step of the herein described process.

Fig. 3 is a similar section of the same fabric after it has been treated to the second step of the herein described process.

Fig. 4 represents a portion of an ornamental fringe which has been treated in accordance with the process embodying the present invention.

Fig. 5 represents an artificial flower which has been treated in accordance with the herein described process.

It is frequently desirable in the manufacture of ornaments of various kinds such as tassels, artificial flowers and the like or of laces and fabrics of various kinds to produce a pleasing effect upon the article or material by treating it in such a manner as to produce a frosted effect in one color or in several colors as desired. The present invention contemplates the provision of an improved process for producing the desired effects by impregnating the fabric or article with a strong solution of a salt in a manner about to be described, the evaporation of the solvent causing the salt to crystallize upon the surface of the fabric thereby producing a frosted or sparkling effect.

In order to accomplish the desired result, an aqueous solution of a salt forming large and beautiful crystals is prepared, the salt being preferably of a non-poisonous nature, 70 a suitable adhesive agent such as gum arabic being added to the solution. The article or fabric to be treated is dipped in the solution and permitted to dry, after which it may again be dipped in the same solution and permitted to dry. The final step involves dipping the article in a suitable coloring solution such as aniline dye which colors the crystals formed by the first steps and thereby produces 75 very beautiful effects.

Preferably the process is carried out by preparing a solution by dissolving say one teaspoonful of gum arabic in two quarts of water, the whole being brought to the boiling point. After the gum arabic has become thoroughly dissolved in the boiling water, one pound of ammonia alum is added, the whole being thoroughly stirred until all of the alum has become dissolved. This procedure produces a hot solution ready for dipping of the fabric or article. While gum arabic and ammonia alum have been specified as the ingredients used in preparing the dipping bath or solution it is not desired to limit the invention to the precise ingredients specified, as any salt which is soluble in hot water may be used. Preferably a salt should be used which forms large crystals and which is very soluble in hot water but only slightly soluble in cold water. Any material equiva-

lent to gum arabic may also be used. The object of the gum arabic is to impregnate the fabric or article with an adhesive agent which will cause the crystals to adhere firmly to the fabric or article after the solvent has evaporated in the drying process. It is necessary of course that the salt and adhesive material used be of a nonpoisonous nature in order to make the crystalline coating on the fabric or article harmless. It is also desirable that the salt and adhesive material be only slightly soluble if at all in cold water so that the crystals will not be readily dissolved from the fabric or article.

After the solution or bath just mentioned has been prepared the ornament, fabric or article which it is desired to coat is dipped in the hot solution and allowed to remain there a few minutes until the article dipped has become thoroughly impregnated with the hot liquid. The article is then removed and allowed to dry. As the liquid adhering to the garment cools and evaporates the concentration of the salt in the solution is gradually increased until the point of supersaturation is reached and passed; wherupon, as the solution still further cools and evaporates, crystals begin to form and at the same time the gum arabic separates out and hardens into a gelatinous binder holding the crystals firmly together and upon the article. Fig. 2 represents diagrammatically a fabric after it has been dipped once and permitted to dry in the manner just described. In this figure the numerals 1 represent the interwoven threads or fibres of the fabric while the numeral 2 represents the crystalline coating adhering to the threads or fibres. This first step produces fine and strongly adhering white crystals which sparkle when held in the light thereby producing a white frosted effect.

The next step is to again dip the article or fabric in the hot solution and again permit it to dry in the manner aforesaid. Fig. 3 illustrates the appearance of a section of fabric after the second coating of white crystalline salt has been formed, the numeral 3 representing the second coating of crystals. After the second dipping, the hot solution again cools and evaporates until the point of supersaturation is reached, whereupon the crystals already present upon the surface of the fabric cause a rapid formation of crystals from the newly added solution with the result that larger and more beautiful crystals will be formed.

As the final step in the process the article or fabric is dipped in a coloring solution in which the crystals are not soluble, such as a solution of an aniline dye and camphor dissolved in alcohol. As a result of this last step the crystals on the article or fabric will be colored according to the color of the dye and by choosing suitable colors very beauti-

ful effects may be produced. The final step in the process is the drying of the fabric or article thoroughly.

The whole result of the foregoing process is that beautiful crystals will be formed which adhere firmly to the article or fabric and are colored in accordance with the dye chosen. By choosing a salt which is readily soluble in hot water but practically insoluble in cold water, crystals may be formed which adhere very firmly and yet are not readily washed off if the article should become moistened, since gum arabic is not easily soluble in cold water.

The foregoing process may be used in a variety of ways to create pleasing effects upon articles, particularly articles composed of woven fabrics or fibrous materials. In Fig. 1 there is shown a butterfly which has been cut from a piece of fabric and dipped in the frosting solution, from which it will be seen that crystals are clinging firmly to the fabric from which the butterfly has been cut. The butterfly shown in Fig. 1 may be made in several ways, one way being to dip the entire butterfly in the solution of ammonia alum, thereby covering the butterfly with white sparkling crystals. After the crystals have been produced, portions of the butterfly's wings may be dipped in various coloring solutions so that each portion of the wings will be given a different color. By folding the butterfly through the center of its body and then dipping the fold including the antennae 4 in a black or brown solution, a butterfly will be produced in which the wings are beautifully colored while the body and antennae will be in black or brown, thereby creating a pleasing effect.

In Fig. 4 there is shown a piece of fringe which has been treated by the process herein described from which it will be observed that there are numerous crystals adhering to the loose threads 5 forming the fringe.

Fig. 5 illustrates an artificial flower which has been treated to the within described process. Each of the petals 6 of the flower may be dipped to form a white frosted coating and afterwards each petal or group of petals may be dipped in a separate coloring solution so that the petals and other parts of the flower when assembled will present a novel and pleasing appearance.

The process may also be used in other ways which will be readily understood from the foregoing brief description to produce a variety of effects. For instance, tassels, laces, or ornaments of various kinds may be treated either wholly or partly by the foregoing process to produce desired color effects, and it is not desired to limit the use of the process to the treating of any one fabric or article.

The hereinbefore described process and a product produced thereby admits of con-

siderable modification without departing from the invention, as the ingredients, proportions, conditions, steps and order of steps may be varied in practice; therefore, it is not wished to be limited to the precise order of operations and details shown and described, which are as aforesaid, by way of illustration merely. In other words the scope of protection contemplated is to be taken solely from the appended claims, interpreted as broadly as is consistent with the prior art.

10 What is claimed as new is:

15 1. A process of the character described which involves first dipping the article to be treated in a hot aqueous solution consisting of gum arabic and ammonia alum, then drying said article whereby said alum crystallizes upon said article and said gum arabic separates and hardens into a binder to firmly hold said crystals together, then again dipping said article in said hot solution, and again drying the article, thereby producing larger crystals, then dipping said article in 25 a coloring solution, and finally drying said article.

20 2. A process of the character described which involves dipping the article to be treated in a hot aqueous solution consisting of gum arabic and ammonia alum, in the proportions of about one teaspoonful of gum arabic to two quarts of water and one pound of ammonia alum, drying said article, whereby said alum crystallizes upon said article, 25 and said gum arabic separates and hardens into a binder to firmly hold said crystals together, again dipping said article in said hot solution, again drying said article thereby forming larger crystals, then dipping said 40 article in a coloring solution consisting of an aniline dye and camphor dissolved in alcohol, and finally drying said article.

45 In testimony whereof I hereby affix my signature.

MARIA LUISA MESA.

50

55

60

65